

## UNITED STATES PATENT OFFICE.

VICTOR LEE EMERSON, OF PHILADELPHIA, PENNSYLVANIA.

## COVERING FOR CONSTRUCTING AIRCRAFT.

No Drawing.

Application filed August 23, 1921. Serial No. 494,688.

*To all whom it may concern:*

Be it known that I, VICTOR LEE EMERSON, a citizen of the United States, residing at Philadelphia, county of Philadelphia, and 5 State of Pennsylvania, have invented a certain new and useful Improvement in Coverings for Constructing Aircraft, of which the following is a specification.

This invention relates to an improved covering for constructing aircrafts, and is particularly adapted to the construction of the wings and bodies thereof.

An object of the invention is to provide a material which will have the qualities of 15 lightness, strength, durability, and be of such character as to be practically transparent to an observer and non-inflammable.

Another object is to provide a covering which will be unaffected by moisture, oils, 20 or gasoline.

The coverings for the purpose herein described now in use deteriorate very rapidly, and when once a tear in the same is started it rapidly enlarges, so as to soon destroy 25 the usefulness of the covering. When in flight the impact of the air against the covering acts to accelerate the destruction of the covering, as when once a tear is started the force of the air acting against the torn 30 portion rapidly enlarges the tear. Such tears are very common in military use from the effect of projectiles. With the use of my invention the danger from destruction of the plane in mid air from this cause is 35 avoided.

It has been heretofore attempted to treat the covering with pigments so as to effect a camouflage when in use for a military purpose. This has not been altogether successfully accomplished with the coverings 40 now in use. Constant inspection, repair, and replacement are necessary, and to this end it is desirable to have the ribs or supporting portions of the plane clearly visible 45 without the removal of the covering. This is impossible when the ordinary airplane cloth treated with a pigment in the usual manner is employed, as this type of covering is opaque.

In my improved covering I employ a 50 metallic netting which may be filled with a transparent coating offering an imperforate surface to the air. While various coatings may be used, I have found that a preparation composed of ammonium bichromate and fish glue is very satisfactory. The 55 chemical action between the ammonium bichromate and fish glue forms a phosphate, and the composition is further acted upon by the actinic rays of light and becomes a 60 hard, transparent coating suitable to the accomplishment of the objects of my invention. I have also found that a coating whose basic constituent is sodium silicate 65 is also very satisfactory. The wire netting used is susceptible of being punctured repeatedly without subject to tear, with resultant destruction, as with the ordinary coverings. This enables the aviator to sustain his flight without danger of destruction of his plane in mid air, 70 upon being struck with projectiles. The netting being covered with the transparent coating, which fills the open spaces therein, presents an almost invisible object from the 75 earth, which makes the plane a very difficult target.

Another object obtained by the use of my improved covering is immunity from fire, 80 as the netting is of a metallic nature and the coating is preferably non-inflammable. Thus the danger from fire is avoided, which is present with coverings composed of inflammable material, as heretofore used. By the use of my invention these great dangers and 85 difficulties of the aviator are avoided. In order to renew the covering it is only necessary to remove the coating and recoat the netting. This saves great expense and is easily and quickly accomplished. Repairs are also possible with a minimum of expense and labor, 90 and a damaged rib or support can be detected without difficulty, due to the transparency of the coating, which would be impossible with the ordinary opaque covering. 95 The covering of my invention is easily applied, and when once in place remains permanently fixed, without stretching or

buckling, as is the case with the ordinary airplane covering now used. My improved covering also adds great strength to an aircraft, being structurally a metallic reinforcement.

Having described my invention, what I claim is:—

As an article of manufacture, a covering for constructing aircrafts, comprising a netting having a coating composition thereon

resulting from the combination of ammonium bichromate and fish glue.

In testimony whereof, I have signed my name to this specification in the presence of two subscribing witnesses, this 19th day 15 of August 1921.

VICTOR LEE EMERSON.

Witnesses:

LAWRENCE S. PADDICK,  
RUSSELL W. SCHIMPF.